

Oct. 29, 1929.

L. JONES

1,733,226

METHOD OF MAKING VALVE CASINGS

Filed April 19, 1924



Fig. 1.



Fig. 2.



Fig. 5.



Fig. 4.



Fig. 5.

Inventor  
*Lloyd Jones*

By *C. C. Osgood*

Attorney

## UNITED STATES PATENT OFFICE

LLOYD JONES, OF FREEPORT, NEW YORK, ASSIGNOR TO THE COLUMBUS MACHINE COMPANY, OF COLUMBUS, OHIO, A CORPORATION OF OHIO

## METHOD OF MAKING VALVE CASINGS

Application filed April 19, 1924. Serial No. 707,583.

The present invention is directed to an improved method for making valve casings.

The primary object of the invention is to produce a method whereby valve casings, particularly gate valve casings, can be produced by the extrusion method in order that the hubs thereof will be integral with the valve casing or body.

A further object of the invention is to provide a valve casing which is extremely light and strong and one which can be manufactured at a minimum cost.

With these and other objects in view, as will appear as the description proceeds, the invention consists in the novel features of construction, combinations of elements and arrangements of parts, and hereinafter to be fully described and pointed out in the appended claim.

In the accompanying drawing:

Figure 1 is a top plan view of the billet used,

Figure 2 is a side view thereof,

Figure 3 is a sectional view showing the billet in the die, the plungers being shown in their inoperative positions,

Figure 4 is a sectional view, the plungers in the positions assumed for extruding the billet, and

Figure 5 is a side view of the completed casing or body.

Referring to the drawing 1 designates the general form of the billet after being subjected to a forging operation, said billet having the same general contour of the die 2.

This die is of the sectional type so that the billet can be easily placed therein for shaping and is of sufficient strength to withstand the pressure to which the billet is subjected.

The billet in its initial or solid form simulates in general the contour of a gate valve casing and in order to extrude the billet to provide a hollow casing a pair of horizontally disposed diametrically opposed plungers

3-3 are employed and a vertically movable plunger 4, said plungers being simultaneously movable to points as shown in Figure 4. These plungers may be reciprocated in any approved manner, but preferably by hydraulic presses (not shown).

As shown in Figure 3 the plungers 3 and 4 are in their inoperative positions and when simultaneously moved the plungers engage the billet 1, treated to an extrusion heat and is subjected to the action of the plungers, whereupon the billet is extruded into the shell form as shown in Figure 4. The movement of the plungers are so regulated that they will reach their respective positions as shown in Figure 3 simultaneously, thus positively extruding the metal into the vertical branch 5 and horizontal branches 6 of the die 2, thereby producing a valve casing wherein the hubs 7 and body 8 are integrally connected. After the billet has been extruded to the form as shown in Figure 4 the resultant shell is removed from the die 2 and the branch 5 and branches 6 are rolled or otherwise suitably manipulated to produce the respective flanges 8' and 9.

It will be of course understood that the confronting or inner ends of the hubs 7 are of sufficient thickness to permit the same to be interiorly threaded for engaging the usual ring seats (not shown) or to provide valve seats 7'.

The billet is preferably formed from metal alloy especially adapted for use in connection with an extrusion method, but it will be understood that metal used in casting may be used and when subjected to the action of the plungers will produce a casing which will not only be light but positively non-porous and especially desirable for use for making valves of this type.

After the billets have been formed into the general shape as shown in Figure 5 it sometimes occurs that fins, webs or other obstructions will remain in the casing at the juncture of its branches and it will be of course understood that these obstructions can be removed by a reamer or in any other suitable manner so that the interior of the completed valve will be unobstructed.

As is well known the gate used in connection with this type of casing is guided to its seats and in order to provide these casings with such guiding means the plunger 4 is provided with grooves 10 upon opposite sides 100

so as to produce guiding ribs 11 during the manufacture of the casings or body.

The light, porous valve casing produced by the extrusion of the billet is what may be properly termed a worked metal casing valve as distinguished from a pierced casing.

What is claimed is:

The method of forming a valve casing having integral hub members which consist in introducing a metal billet into a die having a chamber open at one end and having open-ended lateral chambers communicating with the other end of the main chamber, subjecting the billet to the simultaneous action of a plurality of plungers each introduced through one of said openings while permitting of the unrestricted outward flow of the metal between the plungers and the adjacent wall of the die and thereafter forming flanges on the top of the casing and on the ends of the hub members produced in the extrusion operation whereby a relatively light, non-porous, worked-metal valve casing of homogeneous texture is produced.

In testimony whereof I affix my signature

LLOYD JONES.

30

35

40

45

50

55

60